

## UNITED STATES PATENT OFFICE.

EDWARD S. FARROW, JR., OF ROCHESTER, NEW YORK, ASSIGNOR TO EASTMAN KODAK COMPANY, OF ROCHESTER, NEW YORK, A CORPORATION OF NEW YORK.

## DECOLORIZING CELLULOSIC MATERIAL SUCH AS FILM BASE.

No Drawing.

Application filed March 7, 1923. Serial No. 623,339.

*To all whom it may concern*

Be it known that I, EDWARD S. FARROW, Jr., a citizen of the United States of America, residing at Rochester, in the county of Monroe and State of New York, have invented certain new and useful Improvements in Decolorizing Cellulosic Material Such as Film Base, of which the following is a full, clear, and exact specification.

This invention relates to a process for removing dye from tinted or colored material, such for example as film base or support. One object of the invention is to provide a process for removing dye from such material inexpensively, rapidly and with a minimum number of operations. Other objects will hereinafter appear.

My invention is especially useful when employed in the removal of dye from tinted cellulosic bases of photographic films. One embodiment of it will, therefore, be described in connection with such film by way of example; but the invention is, of course, not limited to this particular illustrative field. Photographic films have come into extensive use, the bases or supports of which contain a colored or dyed layer. The latter may be upon either side of the main support, or many be located throughout the entire cellulosic material.

When scrap or other waste pieces of such colored film base accumulate, it is desirable to reclaim them by removing the color and using the cellulosic addition compounds again. I have discovered that this can be done rapidly, inexpensively and with a minimum of work by dissolving the colored scrap and passing the solution through decolorizing carbon, such as bone-char.

My invention can be employed in the decolorizing of film bases, whether the latter contain cellulose nitrate, cellulose acetate or cellulose ethers, these being typical illustrations of the cellulosic addition compounds to which my process is applicable. At the present time a colored nitrocellulose film base is the one that is most widely used and the specific details chosen for illustration will be directed to the treatment of it.

I dissolve the scrap or waste film base in a suitable solvent which, in the case of a nitrocellulose base, is preferably methyl alcohol or acetone or a mixture of these substances in any relative proportions. In order

to facilitate the solution of the scrap and in order to obtain an uncontaminated product, it is useful to chop up the scrap and wash it with hot water until the gelatinous coatings are removed. The amount of the solvent used for dissolving a given amount of scrap may be varied within wide limits, as will be understood by those skilled in the art. Where the solution of cellulosic material is to flow through a column of bone-char, I find 12 parts by weight of wood alcohol or acetone, or a mixture of them, relative to 1 part of film scrap to be a useful proportion. The scrap and solvent are conveniently charged into any of the well known dope mixers used in this art and agitated until a sufficiently homogeneous solution is obtained. This, of course, will be colored with the dye at this stage.

The solution is then brought into active contact with decolorizing carbon, the interaction being sufficiently thorough to bring each part of the solution into contact with some of the decolorizing material. This can be most conveniently effected in the case of the above described illustrative solution by passing it down through a vertical column or mass of decolorizing bone-char of the type used, for instance, in decolorizing sugar. Of course, other decolorizing forms of carbon may be employed, such as properly activated charcoal. The removal of the dye may take place completely by maintaining the solution in contact with the bone-char for a sufficient length of time, say by providing a long enough column of bone-char. Or the dye may be removed step by step, such as by passing it repeatedly through a mass of bone-char too small to extract the dye at the first contact. In this way a dope which is too colored may be lessened in tint by a partial action of the carbon in accordance with the principles of my invention.

The action takes place sufficiently rapidly to make it unnecessary to heat the materials above ordinary room temperature, although mild heating will, of course, assist the flowable qualities of the dope. When the carbon, such as bone-char, has its activity lessened through taking up large quantities of dye, it may be revived by heating or charring out of contact with the air by the usual methods well known to those skilled in the art. This restores the activity of the ma

terial and at the same time destroys the dye previously adsorbed or taken up by it. The process has been found to operate successfully with a large variety of both basic and acid dyes.

Having thus described my invention, what I claim as new and desire to secure by Letters Patent is:

1. The process of decolorizing a dyed cellulosic addition compound, which comprises dissolving said compound and treating the solution with decolorizing carbon.

2. The process of decolorizing a dyed cellulosic addition compound, which comprises mixing said compound with sufficient solvent to form a flowable solution and passing said solution through decolorizing bone-char.

3. The process of decolorizing dyed nitrocellulose, which comprises bringing said nitrocellulose into solution and bringing said

solution into active contact with decolorizing carbon.

4. The process of decolorizing dyed nitrocellulose, which comprises mixing said compound with sufficient solvent to form a flowable solution and passing said solution through decolorizing bone-char.

5. The process of decolorizing dyed nitrocellulose film base, which comprises dissolving 1 part thereof by weight in 12 parts by weight of volatile solvent and passing the solution through decolorizing carbon.

6. The process of decolorizing dyed nitrocellulose film base, which comprises dissolving it in a mixture containing wood alcohol until a flowable solution is obtained and flowing said solution through a column of decolorizing bone-char.

Signed at Rochester, New York, this 26th day of February, 1928.

EDWARD S. FARROW, Jr.